

Jan. 17, 1928.

1,656,843

E. STRAUB

PROCESS FOR PHOTOGRAVURE

Filed March 26, 1926



Inventor  
Emile Straub.

By William C. Linton  
Attorney.

## UNITED STATES PATENT OFFICE.

EMILE STRAUB, OF PARIS, FRANCE, ASSIGNOR TO JEAN GRIFFITHS, OF PARIS,  
FRANCE.

## PROCESS FOR PHOTOGRAVURE.

Application filed March 26, 1926, Serial No. 97,803, and in France February 10, 1926.

The invention relates to improvements in processes for photogravure upon zinc plates for printing purposes.

The said improvements have for their objects the composition of the products and the method of utilizing the same.

As a whole, my said process differs from the known processes by the composition of the mixtures and also from the fact that the 10 zinc plate does not require to be treated in different baths. In this manner I obtain the following advantages.

The operator can now develop the plate with great accuracy, stopping the action 15 when the image appears or further treating the parts of the image which require a greater development. Since it will now suffice to rub the plate with the various products which can be preliminarily prepared, 20 no great installation is required, and the operations can be performed in an ordinary room upon a small table, and by a person possessing little skill.

In the known processes, the drawing or 25 design must be made upon a special paper, but my said process provides for the copying or an original, whether printed, written or drawn, upon any kind of paper, and even of the thickness of Bristol board. It is not 30 necessary that the lines of the original shall be perfectly black.

The following description taken in connection with the accompanying drawing clearly shows the manner in which my said 35 process is carried into effect, as well as the composition of the products in use.

Fig. 1 shows the zinc plate covered with the emulsion used.

Fig. 2, shows the zinc plate covered with 40 the emulsion and with the design to be reproduced.

Fig. 3 shows the zinc plate covered with emulsion after development and after the soluble parts have been dissolved.

Fig. 4 shows the zinc plate with a gum 45 covering the bare spots of the zinc shown in Fig. 3.

Fig. 5 shows the zinc plate with the emulsion removed and the parts inked.

Fig. 6 shows the zinc plate ready for use 50 in printing.

The plate is first cleaned by rubbing it with rather coarse powdered pumice stone

and with dilute sulphuric acid (5 grams per 500 grams water).

1st operation.—The plate is covered with a sensitive layer, and for this purpose a small quantity of the following mixture is spread upon the zinc plate with a pad: Water 125 grams, gum arabic 30 grams, ammonium bichromate 6 grams.

The zinc is then dried by means of hot air electric dryer. The drawing (or letter) to be reproduced, which has been formed upon any kind of paper, is pressed against the zinc plate, and the whole is exposed to the light, using for instance a strong incandescent lamp. In Fig. 1, *a* indicates the zinc plate, *b* the sensitive layer, and in Fig. 2 the object to be reproduced is indicated by *c*, 70 the parts in black being indicated in black.

2nd operation.—A few drops of the following solution: Water 150 grams, glycerin 400 grams, acetic acid, crystallizable 25 c.c., are placed upon the zinc plate, and it is then 75 rubbed with a soft pad (printers' blanket) until the image appears, bearing particularly on the parts which appear more slowly. The plate is then wiped with a soft cloth. Fig. 3 represents the zinc plate with emulsion after development, the soluble parts (corresponding to the black parts of the design) are indicated by *d* and the insoluble parts (corresponding to the light parts of the design) by *e*.

3rd operation.—The plate is washed with a few drops of the following solution: Alcohol, denatured (90 per cent) 470 c.c.; acetic acid, commercial 30 c.c., and this will complete the development, even slightly attacking the zinc in the parts unacted upon by the light (blacks of the drawing). This washing removes the remainder of the emulsion which was not altered by the action of the light.

4th operation.—A small quantity of the following solution: Alcohol, denatured (95 per cent) 475 c.c.; shellac, brown 25 grams, is spread upon the zinc with a soft cloth, rubbing in such manner that the shellac will 100 penetrate into the parts of the plate where the zinc is left bare (blacks of the drawing). The plate is then dried with an electric dryer employing cold air, and is then washed in ordinary water and dried. In Fig. 4 the 105 gummed parts are indicated by *f*. The gum

acts as a bond between the zinc and the ink which is applied in the following operation.

5th operation.—The zinc plate is inked with a pad containing a small amount of printers' ink mixed with turpentine. The plate is then dried by hot air. The ink takes hold upon the zinc, that is the parts covered by the shellac, and not upon the emulsion which always remains somewhat moist.

10 6th operation.—The zinc plate is rubbed over with a small amount of talcum powder to dry the ink.

7th operation.—The insoluble emulsion formed upon the plate is removed by a soft cloth, and I employ the following solution for this removal: Hydrochloric acid 25 c.c., water 1 liter. Should there be any defects in the drawing, these are to be retouched. In Fig. 5 it is seen that all the emulsion is

20 lifted from the zinc plate and that there remains only the inked parts indicated by *f*.

8th operation.—In order to attack or to etch the plate in the parts which are not to be inked, the plate is coated with a brush 25 made of textile fabric, with the following solution: Hydrochloric acid 35 c.c., nitric acid 35 c.c., phosphoric acid 20 c.c., gallic acid 4 gram. The zinc plate is then wiped and dried, and it is now ready for the 30 printing process. The press, or a roller machine, can produce any desired number of copies of the original drawing or letter. In Fig. 6, the parts attacked by the acid and

roughened are indicated by *g*, while the smooth parts which retain the ink are indicated by *h*.

Obviously, the proportions above indicated for the composition of the products are susceptible of all necessary modifications, without departing from the invention.

Having so described my said invention and in what manner it is performed, I declare that what I claim is—

The process for forming etched plates for use in printing which comprises applying to the plate a thin layer of a solution of gum arabic and ammonium bichromate, drying it and exposing the surface to the action of light through the object to be reproduced, rubbing the exposed plate with a solution of 50 glycerine, water and acetic acid until the image appears, washing the plate thereafter with a solution of alcohol and acetic acid, applying to the plate a solution of a quickly 55 drying varnish and rubbing in order to make the varnish penetrate the parts of the plate where the plate is bare, thereafter drying and washing and inking it with printing ink, thereafter removing the light affected 60 layer with dilute hydrochloric acid and etching the exposed parts of the plate.

In testimony whereof, I have signed my name to this specification at Paris, this 10th day of March, 1926.

EMILE STRAUB.